

## UNITED STATES PATENT OFFICE.

WIRT D. RIAL, OF WATSON, AND WHITFORD R. BARRATT, OF PALOS VERDES ESTATES, CALIFORNIA, ASSIGNEES TO PAN AMERICAN PETROLEUM COMPANY, OF LOS ANGELES, CALIFORNIA, A CORPORATION OF CALIFORNIA.

## PROCESS OF PURIFYING AND ADDING A GREEN FLUORESCENCE TO LUBRICATING OIL.

No Drawing.

Application filed June 7, 1927. Serial No. 197,225.

This invention relates to a method of neutralizing, imparting a green fluorescence, clarifying, and improving the color of lubricating oil; and is a continuation in part of 5 the application of John C. Black, Wirt D. Rial and John R. McConnell, Serial No. 141,424, filed October 13, 1926, "process of imparting fluorescence to oil," which reveals a method of clarifying, improving the color 10 and imparting a desired fluorescence to an oil. In that pending application the process involves mixing coal tar pitch and a decolorizing clay with a lubricating oil stock, then heating the same in a commingled state 15 at a suitable temperature for obtaining the desired fluorescence and color, and thereafter separating the oil from the decolorizing clay, adsorbed constituents, and coal tar residue. 20 We have discovered that while that method produces a satisfactory product, the decolorizing clay cannot be commercially revivified for re-use, and also that a smaller quantity of the decolorizing clay may be 25 employed by our improved method for obtaining the desired color and fluorescence of a lubricating oil stock.

An object of the invention is to provide a 30 method or process whereby a substantially uniform clarified oil of the desired color and fluorescence may be produced with a minimum consumption of the clarifying and decolorizing agent; another object is to provide such a process that the decolorizing 35 agent may be recovered for re-use and the process conducted with a minimum consumption of time.

The process of this application consists broadly, first in the separation of lubricating oil from crude petroleum oil by a distillation operation, preferably under a reduced pressure less than atmospheric, then immediately treating the separated lubricating oil stock at an elevated temperature under 45 steam pressure with a solution of caustic potash as described in the pending application of John C. Black and Wirt D. Rial, Serial No. 187,110, filed April 27, 1927. The lubricating oil stock after this treatment is 50 then treated with sulfuric acid by well-known methods followed by treatment with an adsorbent clay to substantially completely remove the acid reaction products as out-

lined in United States patent of James W. Weir, No. 1,564,501.

After these treatments the lubricating oil stock is re-distilled, preferably under a pressure less than atmospheric, to separate therefrom the heavier cylinder lubricating oil stock from the relatively lighter grades of 60 lubricating stock, known in refinery practice as "overhead stock." The "overhead stock" which may be any desired grade, is commingled with a mixture of coal tar and lime, preferably hydrated lime, after which the 65 commingled products are heated to approximately a temperature of 250° F. and then filtered. The amount of coal tar pitch and lime employed is approximately 1 1/4 per cent 70 coal tar pitch and 1/8 of a pound of lime (Ca(OH)<sub>2</sub>) per gallon of oil treated. After separating the lime and residual coal tar pitch from the treated lubricating oil stock, preferably by a filtration operation, the oil 75 is clarified and decolorized with a decolorizing clay at temperatures ranging from 230 to 320° F. or a little higher. The amount of coal tar pitch may vary from as low as 1/2 to as high as 5 per cent by weight of the oil treated, this variation depending upon 80 the stock treated and the product desired. In case it is desired to obtain a more intense green fluorescence to the lubricating oil stock, a greater percentage of the coal tar is employed in accordance with the fluorescence desired, and in which case a larger 85 proportional percentage of lime may be employed in order to retain the residual coal tar pitch, which may vary from 1/10 of a pound to as high as 1 pound per gallon of 90 oil to be treated.

As a specific example of a pitch which may be employed, a coal tar pitch made by the distillation of a coal tar may be given as an illustration. This pitch may be a reduced 95 residue of varying viscosities, preferably however, a pitch which does not contain hydrocarbons having boiling points less than the lubricating oil stock treated, is desired.

It is to be understood that any lubricating oil stock may be treated by this invention which may or may not have been treated by the methods heretofore described in this invention and that such invention consists principally in the combined treatment of a 100 lubricating oil stock with lime, preferably 105

calcium hydroxide and a coal tar residuum containing hydrocarbons having boiling point substantially not less than the lubricating oil to be treated, that by such method 5 the lubricating oil stock treated is rendered free of acid impurities as well as imparting thereto a desired green fluorescence, this treatment being carried out preferably at temperatures substantially not less than 10 230° F.

While the process herein described is well adapted for carrying out the objects of the present invention, it is to be understood that various modifications and changes may be 15 made without departing from the spirit of the invention and the invention includes all changes and modifications as appear in the scope of the appended claims.

We claim:

- 20 1. A process of purifying and improving the quality of lubricating oil containing acid constituents, comprising commingling the lubricating oil with calcium hydroxide and a coal tar pitch containing green fluorescent bodies at a temperature of substantially not less than 230 degrees F. in quantities sufficient to neutralize and adsorb the acid constituents contained therein and add green fluorescent bodies to the lubricating oil and 25 then separating the lubricating oil containing the green fluorescent bodies from the coal tar pitch residue, and excess calcium hydroxide containing the adsorbed constituents.
- 30 2. A process of purifying and improving the quality of lubricating oil containing acid constituents comprising commingling the lubricating oil with calcium hydroxide and a coal tar pitch containing green fluorescent bodies at a temperature of substantially not less than 230 degrees F., in quantities sufficient to neutralize and adsorb the acid constituents contained therein and add green 35 fluorescent bodies to the lubricating oil and then separating the coal tar pitch residue and excess calcium hydroxide containing the adsorbed constituents.
- 40 3. A process of purifying and improving the quality of lubricating oil containing acid constituents comprising commingling the lubricating oil with calcium hydroxide and a coal tar pitch containing green fluorescent bodies at a temperature of substantially not less than 230 degrees F., in quantities sufficient to neutralize and adsorb the acid constituents contained therein and add green 45 fluorescent bodies to the lubricating oil and then separating the coal tar pitch residue

and excess calcium hydroxide containing the adsorbed constituents from the lubricating oil containing the green fluorescent bodies, and finally clarifying and decolorizing the lubricating oil to the required degree with a 50 clarifying and decolorizing clay.

3. A process of purifying and improving the quality of lubricating oil containing acid constituents comprising commingling the lubricating oil with substantially dry calcium hydroxide and a coal tar pitch containing green fluorescent bodies at a temperature of substantially not less than 230 degrees F., in quantities sufficient to neutralize and adsorb the acid constituents contained therein and add green fluorescent bodies to the lubricating oil and then separating the coal tar pitch residue and excess calcium hydroxide containing the adsorbed calcium salts from the lubricating oil and green fluorescent bodies and finally clarifying and decolorizing the lubricating oil to the required degree with a clarifying and decolorizing agent.

4. A process of purifying, improving the quality and adding green fluorescent bodies to a lubricating oil containing acid constituents, comprising commingling the lubricating oil with calcium hydroxide and a coal tar pitch at a temperature of substantially not less than 230 degrees F. in quantities sufficient to neutralize and adsorb the acid constituents contained therein and add green fluorescent bodies to the lubricating oil and then separating the coal tar pitch residue and excess calcium hydroxide containing the adsorbed constituents from the lubricating oil containing the green fluorescent bodies, and finally clarifying and decolorizing the lubricating oil to the required degree with a clarifying and decolorizing agent.

In testimony whereof we affix our signatures.

WIRT D. RIAL.  
WHITFORD R. BARRATT.